

# United States Patent [19]

Lindberg et al.

[11] 3,856,360

[45] Dec. 24, 1974

[54] ALUMINUM BASE ALLOY DIE CASTING  
WHEEL

3,128,176 4/1964 Martin ..... 75/148  
3,199,979 8/1965 Martin ..... 75/142

[75] Inventors: **Richard S. Lindberg**, Homewood;  
**G. Leslie Armstrong**, Crete, both of  
Ill.

Primary Examiner—R. Dean  
Attorney, Agent, or Firm—Dressler, Goldsmith,  
Clement & Gordon, Ltd.

[73] Assignee: **U.S. Reduction Co.**, East Chicago,  
Ind.

[22] Filed: **Mar. 1, 1973**

[21] Appl. No.: **337,002**

## Related U.S. Application Data

[62] Division of Ser. No. 85,372, Oct. 30, 1970, Pat. No.  
3,726,672.

[52] U.S. Cl. .... **301/65, 75/142**

[51] Int. Cl. .... **B60b 1/08, C22c 21/02**

[58] Field of Search .... **75/140, 141, 142, 148,  
75/146, 301/5, 65, 96; 148/32, 32.5**

## References Cited

### UNITED STATES PATENTS

2,823,995 2/1958 Blackmun ..... 75/148

## [57] ABSTRACT

An aluminum base alloy and an automobile wheel die-cast therefrom, the alloy consisting essentially of aluminum and by weight percentage of the total composition, magnesium 0.25 to 0.6%, copper 0.25 to 0.6%, iron 0.5 to 1.5%, silicon 11 to 13.5%, chromium 0.25 to 0.4%, a maximum of 3% zinc, a maximum of 0.5% manganese and a maximum of 0.2% of each of titanium, nickel, tin and lead.

2 Claims, 2 Drawing Figures



PATENTED DEC 24 1974

3,856,360

FIG. 1



FIG. 2



## ALUMINUM BASE ALLOY DIE CASTING WHEEL

This is a division of application Ser. No. 85,372, filed Oct. 30, 1970, now U.S. Pat. No. 3,726,672.

This invention relates to an aluminum base alloy having high strength, excellent die-casting characteristics, excellent machinability and superior mechanical properties. It is especially useful for the die casting of automobile wheels, although its application is not so limited.

With the advent of a keen interest in the use of lightweight aluminum base alloys for articles which must stand the abuse and stresses heretofore reserved for ferrous metals and alloys, it became important to develop improved aluminum base alloys for such products. However, to be maximally useful for automobile wheels and other such products, aluminum base alloys had to be die-castable, corrosion resistant, readily machinable and of a higher strength than those aluminum base alloys previously available and at a lower cost than other available alloys having comparable properties.

Although aluminum base die-cast alloys have been on the market for many years where lightweight, accurate dimensioning and the like was important, generally those alloys were not suitable for use in applications where substantial abuse and high stresses were encountered.

The only alloy which met with limited success in, and which has properties generally suitable for high stress applications, such as in die-cast automobile wheels, is one known to the trade as "364 alloy." This is made generally in accordance with Blackmun U.S. Pat. No. 2,823,995. Although that alloy improved upon prior art alloys in certain respects, the properties of that alloy were not as good as was desirable. Furthermore, the cost of that alloy was too high for general use. Consequently, insofar as aluminum base alloy die-cast automobile wheels were concerned, that alloy was used only for high cost specialty wheels.

In accordance with this invention an aluminum base die-casting alloy having substantially improved mechanical properties is provided. Its cost is substantially lower than the cost of the 364 alloy previously used for similar purposes, and indeed scrap aluminum and other secondary aluminum available for secondary reformulation, rather than primary aluminum, may be used to compound the alloy of this invention. As such, the alloy of this invention provides the commercial potential, for the first time, for the substitution of aluminum base

by weight of the final alloy, 0.25 to 0.6% magnesium; 0.25 to 0.6% copper; 0.5 to 1.5% iron; 11 to 13.5% silicon; and 0.25 to 0.4% chromium. The high silicon content and the copper content substantially contribute, we believe, in combination with the other ingredients to the superior physical properties of this alloy.

The composition of this invention which maximizes the characteristics and properties of die-cast products, such as automobile wheels, while minimizing the costs attendant the manufacture and use of the alloy composition, consists essentially of aluminum, and by weight of the final alloy, 0.25 to 0.6% magnesium, 0.25 to 0.6% copper, 0.5 to 1.5% iron, 11 to 13.5% silicon, 0.25 to 0.4% chromium, a maximum of 3% zinc, a maximum of 0.5% manganese, and a maximum of 0.2% each of titanium, nickel, tin and lead. Die-cast products such as automobile wheels cast of this alloy have an overall combination of impact strength, fatigue strength, tensile strength, yield strength and ductility characteristics which is superior to those of other aluminum base die-casting compositions of which we are aware, including those characteristics available in products die-cast from 364 alloy. Furthermore, the corrosion resistance and machinability of wheels die-cast of this alloy are quite excellent and the die-casting characteristics are as good as any aluminum alloy available for the high stress applications for which the alloy of this invention is useful.

Although the advantages of this invention may be obtained within the aforementioned ranges, we have determined that an especially useful preferred range of ingredients is a composition consisting essentially of aluminum, and by weight of the final composition 0.25 to 0.4% magnesium, 0.25 to 0.5% copper, 0.4 to 0.8% iron, 11 to 12% silicon, 0.3 to 0.4% chromium, a maximum of 1% zinc, a maximum of 0.35% manganese, a maximum of 0.05% of each of titanium and nickel, and a maximum of 0.1% of each of tin and lead.

FIGS. 1 and 2 illustrate typical automobile wheels which have been die-cast with aluminum base alloys.

Die-cast automobile wheels have been made from aluminum base alloys of this invention, as well as from a commercially available 364 alloy. Several such wheels have been analyzed to determine their final composition. Further, those wheels have been tested for yield strength, tensile strength and ductility.

Spoke wheels 10 die-cast generally in the configuration of FIG. 1 were analyzed and were found to have the following compositions (the remainder being aluminum):

|           | Mg  | Cu  | Fe  | Zn  | Si    | Mn  | Ti  | Ni  | Cr  | Sn  | Pb  | Be    |
|-----------|-----|-----|-----|-----|-------|-----|-----|-----|-----|-----|-----|-------|
| 364 Alloy | .25 | .07 | .61 | .04 | 8.63  | .01 | .01 | .01 | .39 | .02 | .01 | .0053 |
| A Alloy   | .32 | .32 | .57 | .29 | 11.64 | .17 | .03 | .01 | .40 | .01 | .01 | 0     |

alloy automobile wheels for steel wheels on a much larger scale.

As its essential ingredients, the die-casting aluminum base alloy of this invention comprises aluminum, and

Test bars were cut from those wheels and flange 12 test bars, spider 14 test bars, and rim 16 test bars were tested for yield strength, for tensile strength, and for percent elongation with the following results:

|                           | Flange<br>A<br>364 | Spider<br>A<br>364 | Rim<br>A<br>364 |
|---------------------------|--------------------|--------------------|-----------------|
| Yield Strength<br>(psi)*  | 18,400             | 15,000             | 20,500          |
| Tensile Strength<br>(psi) | 25,500             | 20,300             | 28,000          |
| % Elongation              | 2%                 | 1 1/2              | 5               |
|                           | 3 1/2              | 2                  | 2 1/2           |

\*Offset equals 0.2 percent

In these characteristics wheels die-cast from an alloy A of this invention were essentially equal to or substantially better than those die-cast from 364 alloy, and at a substantially lesser overall cost. The machinability, the die-casting characteristics and the corrosion resistance of the alloy A of this invention also were all at least as good as, and in some instances substantially better than those of the 364 alloy.

Deep dish wheels 20 die-cast generally in the configuration illustrated in FIG. 2 were also tested for their yield strength, tensile strength and percent elongation. Test bars cut from flanges 22, rims 24 and spiders 26 from alloys B falling within the preferred range of this invention identified above and from a commercially available 364 alloy had the following properties:

|                           | Flange           |        | Spider           |        | Rim              |        |
|---------------------------|------------------|--------|------------------|--------|------------------|--------|
|                           | B                | 364    | B                | 364    | B                | 364    |
| Yield Strength<br>(psi)*  | 22,000<br>18,300 | 16,800 | 23,300<br>17,900 | 17,400 | 23,400<br>19,700 | 19,100 |
| Tensile Strength<br>(psi) | 23,800<br>25,000 | 20,700 | 29,500<br>27,700 | 24,700 | 25,400<br>24,600 | 20,000 |
| % Elongation              | 2½<br>5          | 2½     | 3<br>4           | 3½     | 3<br>4           | 2      |

\*Offset equals 0.2 percent

These last tests from three die-cast wheels, two cast from alloys B of this invention and one cast from 364 alloy even more graphically illustrate the substantially improved characteristics and properties of the alloys of this invention as compared with those of the 364 alloy.

What is claimed is:

1. A die-cast aluminum automobile wheel having a flange, spiders and a rim, said wheel consisting essentially of aluminum, and by weight percentage of the total composition, magnesium 0.25 to 0.6%, copper 0.25 to 0.6%, iron 0.5 to 1.5%, silicon 11 to 13.5%, chromium 0.25 to 0.4%, a maximum of 3% zinc, a maximum of 0.5% manganese and a maximum of 0.2% of each of titanium, nickel, tin and lead.
2. A die-cast aluminum automobile wheel having a flange, spiders and a rim, said wheel consisting essentially of aluminum and by weight percentage of the total composition, magnesium 0.25 to 0.4%, copper 0.25 to 0.5%, iron 0.4 to 0.8%, silicon 11 to 12%, chromium 0.3 to 0.4%, a maximum of 1% zinc, a maximum

of 0.35% manganese, a maximum of 0.05% of each of titanium and nickel and a maximum of 0.1% of each of tin and lead.

\* \* \* \* \*